

July 20, 1943.

J. SUSSKIND

2,324,889

METHOD OF MAKING SHOE HEELS

Filed Dec. 3, 1941



Fig. 5.



Fig. 2. Fig. 3. Fig. 1. Inventor

Julius Susskind

By

Clarence O'Brien

Attorney



Fig. 4.

Patented July 20, 1943

2,324,889

# UNITED STATES PATENT OFFICE

2,324,889

## METHOD OF MAKING SHOE HEELS

Julius Susskind, Brookline, Mass., assignor of  
one-half to Harry Freedman, Boston, Mass.

Application December 3, 1941, Serial No. 421,496

1 Claim. (Cl. 12—147)

My invention relates to improved method of making cushion heels and heel-lifts for shoes, and the primary object of the invention is to economically and efficiently produce a superior product of this character.

Other important objects and advantages of my invention will be apparent from a reading of the following description and the appended drawing wherein for illustrative purposes a preferred embodiment of the invention is shown.

In the drawing—

Figure 1 is a fragmentary side elevational view showing the step or pressing together the combination of heel body, layer of cement, and Celluloid top plate preceding the drying step which imparts the concavo-convex form to the finished product.

Figure 2 is a top plan view of the finished product.

Figure 3 is a transverse internal view along the line 3—3 of Figure 2.

Figure 4 is a side elevational view of the finished heel.

Figure 5 is a fragmentary sectional elevational view showing the heel installed on a shoe.

The present application is a continuation in part of my co-pending application Serial No. 326,092, filed March 26, 1940, for Cushion heel.

The present cushion heel or heel lift 5 comprises the flexible, compressible rubber or similar material body 6 providing the cushioned engagement with the pavement 7 when secured by nails 8 or the equivalent to the heel portion 9 of the shoe 10. The heel 5 further comprises the Celluloid or similar material top plate 11 which is concavo-convex in form and secured by cement 12 to the top of the body 6 in a manner to impart a similar curvature or concavo-convex form to the body 6 and thereby provide a cushion heel which is relatively more flexible and compressible and therefore of greater cushioning effect. In addition, the convexity of the bottom 13 of the heel provides for a more natural and adaptable engagement of the heel with the pavement in walking than is provided by flat bottom heels. The foot rarely comes down on the pavement at the same angle even where the pavement is smooth and level, but usually engages the pavement at an angle and scuffs the edges of the heel before the bottom of the heel finally rests on the pavement, thereby prematurely wearing the heel. In the case of the present invention, however, the edge of the heel engages the pavement at a more obtuse angle due to the convexity of the heel bottom, and settles more

quickly to rest on the pavement because of the greater conforming characteristics inherent therein enabling the heel to flex upwardly as the weight is placed thereon and quickly achieve a full supporting engagement with the heel portion 9, wherein the full support of the ordinary cushion heel is obtained.

In making the present heels, the heel body 6 is cut from flat rubber or similar material plate 10 and is in flat form until further processed as described below. The Celluloid or similar material top plate 11 is likewise cut from flat plate material, and it is of the same size as the top of the heel body 6.

15 The upper surface of the heel body and the lower surface of the top plate 11 are then roughened by any suitable means to better accommodate cement.

16 The upper surface of the heel body is then given a preliminary coating of Celluloid cement which is allowed to dry and then recoated with the same cement as at 12. In the meantime, the lower surface of the Celluloid top plate 11 is washed with a solvent to soften it and adapt it 20 to bond with the Celluloid cement 12 dried on the heel body, the solvent consisting of 50% of acetone and 50% of synthetic methanol.

25 The top plate 11 and the heel body 6 are then registered and placed between two flat pressure plates or blocks 14, 15 and squeezed together. The amount of pressure applied and the duration of this operation depend to some extent on the materials employed, but the top plate 11 and heel body 6 remain in the described situation 30 for several hours or until a satisfactory union between them is achieved.

35 The combination is then removed from the press, trimmed and polished and painted as may be desired.

40 The heels are then laid aside for three or four days, during which time the Celluloid top plate 11 dries and shrinks and both the top plate and the heel body as a result take on the desired uniform concavo-convex contour shown as described.

45 The above mentioned cement is preferably made by dissolving about 1 pound of Celluloid film in 3 gallons of acetone, and after about three days mixing with the resultant about 1½ gallons of wood alcohol and ½ gallon of methyl chloride.

50 Although I have described and set forth herein preferred embodiments of my invention, it is to be understood that I do not wish to limit the 55 application of the invention thereto, except as

may be required by the scope of the subjoined claim.

Having described the invention, what is claimed as new is:

A method of making a cushion heel, said method consisting in providing a Celluloid top plate and a rubber heel body of substantially the same plan shape, softening the top plate with Celluloid solvent, securing the top plate to the upper

surface of the heel body with cement, pressing the top plate and heel body together to complete the union therebetween, removing the pressure from the united top plate and heel body and allowing the same to stand until the Celluloid top plate dries and warps into a permanent concavo-convex form with which the heel body conforms.

JULIUS SUSSKIND.